

## UNITED STATES PATENT OFFICE

HERBERT TRÖGER, OF PLÄUEN, GERMANY

## TANNING FOR THE PRODUCTION OF LEATHERS OF VARIOUS KINDS

No Drawing. Application filed July 28, 1927, Serial No. 209,158, and in Germany February 24, 1926.

My invention relates to the art of tanning hides and skins.

Its object is to provide new and efficient means for reducing the time required for the 5 tanning processes and for improving at the same time the quality of the tanned products so as to obtain only uniformly and thoroughly tanned leathers which are soft and impervious to water.

10 According to my invention, fermenting organisms are added to the tanning liquor; the tanning liquor containing the hides to be treated is alternately subjected to pressure and to vacuum in sequence and, moreover, the 15 hides are subjected to the action of an electric current during the tanning operation.

The first step above-mentioned is carried out by inoculating the tanning liquor with yeast, such as brewer's yeast, or bacteria 20 adapted to support and stimulate fermentation; said bacteria may be raised on organic or inorganic substances such as wheat-gluten-starch, sodium-thiosulphate ( $Na_2S_2O_3$ ) etc.

The above-mentioned fermenting agents 25 are preferably added progressively in small doses to the tanning liquor while being made viz. before the liquor is used for tanning or else may be added during the tanning process proper.

30 The total quantity of the fermenting agents to be added may vary to from 0.25% to 35% of the weight of the liquor consistent with the concentration and fermenting efficiency of the respective agent, and the depletion of the 35 tanning-liquor during the tanning process is compensated by adding ground tanning substances.

After the raw depilated hides or skins have 40 been placed in the tanning vessel—preferably hung up on ropes or chains in the latter—the air is pumped out of the vessel and the tanning liquor, mixed with stimulating agents as above set forth, is subsequently admitted into the vessel, while the latter is kept under 45 vacuum.

After the liquor has been allowed sufficient time to impregnate the material under treatment air is admitted into the tanning vessel and is compressed therein to a pressure of several atmospheres. The contents of the vessel 50

are then alternately subjected to a vacuum and to air pressure in sequence until the tanning is completed.

During the tanning operation, the hides and skins suspended in the bath are subjected 65 to the action of an electric current.

Direct or alternating current may be used for this purpose at a pressure of about 20-35 volt consistent with the size of the tanning-vessel. Voltage and amperage of the current 60 may of course be varied according to circumstances. The current is led to the bath by electrodes which are preferably made of hard-lead, alloyed with antimony, or other substances adapted to stand the chemical attacks 65 of the tanning liquor and their admixtures.

The tanning operation may be carried out either in revolving drums or in stationary drums or containers. Steam may advantageously be introduced into the liquor, during 70 the tanning operation.

What I claim is:

1. A method for tanning hides which consists in suspending the hides in a tanning liquor inoculated with fermentation organisms, creating in the tanning container pressure alternately below and above atmospheric pressure, and causing an electric current to flow through the tanning liquor during the tanning operation. 75

2. A method for tanning hides and skins which consists in suspending the hides in a tanning liquor containing fermentation organisms, creating in the tanning container pressures alternately below and above atmospheric pressure, and causing an electric current to flow through the tanning liquor during 85 the tanning operation.

3. A method for tanning hides according to claim 2, in which steam is introduced into 90 the tanning liquor during the tanning operation.

In testimony whereof I have signed my name to this specification.

HERBERT TRÖGER. 95